

1

3,153,622

## IRRADIATION OF LUBRICATING OILS

Earl L. Humphrey, Verona, and Joseph J. McGrath, Monroeville, Pa., assignors to Gulf Research & Development Company, Pittsburgh, Pa., a corporation of Delaware

No Drawing. Filed Oct. 27, 1959, Ser. No. 848,895

2 Claims. (Cl. 204—154)

This invention relates to procedure for preparing an improved lubricating oil and in particular an improved oil for lubricating aircraft turbines and the like.

Lubricating oils which are presently available are not entirely satisfactory for use under severe conditions, particularly under high temperature conditions. The United States Air Force has required that oils for certain uses such as aircraft turbines meet specifications set forth in Specification MIL-L-9236A. This specification includes a test generally known as the panel coking test and measures the tendency of a lubricating oil to deposit coke at high temperatures. Few lubricating oils give satisfactory coke panel tests.

This invention has for its objective to provide improved lubricating oils. A still further object is to provide procedure for preparing lubricating oils having a low tendency to deposit coke during panel coking tests. A still further object is to provide an improved lubricating oil having a viscosity in the range between about 50 and 150 S.U.S. at 210° F. Other objects will appear hereafter.

These and other objects of our invention are accomplished by subjecting a lubricating oil having a viscosity between about 50 and 150 S.U.S. at 210° F. and which has been treated with hydrogen to the influence of ionizing radiation of between about 0.001 and 10 watt hours per gram of said lubricating oil.

The charge stock employed in our process may be derived from any type of petroleum such as Pennsylvania, Mid-Continent, West Coast, Middle-East crudes, etc. The charge stock must, after the hydrogen treatment, have a viscosity between about 50 and 150 S.U.S. at 210° F. The viscosity of the starting material prior to the hydrogen treatment must be selected so that the product, after the hydrogen treatment, will have the required viscosity of between about 50 and 150 S.U.S. at 210° F. Mild hydrogen treatment does not alter the viscosity of a lube oil stock to a great extent and when such hydrogen treatment is employed, the viscosity of the charge to the hydrogen treatment may be about the same as the required viscosity for the hydrogen treated product, i.e. between about 50 and 150 S.U.S. at 210° F. On the other hand, many hydrogen treatments result in moderate or even extensive reduction in the viscosity of the hydrogen treated product and in such cases the viscosity of the charge to the hydrogen treatment must be proportionately higher so that the product will have the required viscosity after the more or less extensive lowering of viscosity during the hydrogen treating. The charge stock having approximately 50 to 150 viscosity at 210° F. need not be a purified fraction. Thus it is entirely satisfactory to charge to the hydrogen treatment a residual fraction or a distillate fraction which contains the required 50 to 150 viscosity portion as well as other hydrocarbons. If such a mixed charge stock is used the required viscosity portion will be separated, preferably by vacuum distillation before, or after the irradiation.

The hydrogen treatment applied to the above discussed charge stock may be any of the well known hydrogen treatments which are applied to lubricating oil stocks in order to provide improved lubricating oils. In general, the hydrogen treatment is carried out at a pressure between about 200 and 10,000 p.s.i.g.; a temperature between about 400° and 850° F.; at a space velocity be-

2

tween about 0.1 and 16 volumes of charge stock per volume of catalyst per hour; and at a hydrogen recycle rate of between about 400 and 20,000 standard cubic feet per barrel of charge. One known method of hydrogen treating lubricating oils is a mild type of operation to effect decoloration and hydrogenation of easily hydrogenated materials such as olefins. This procedure gives very little if any improvement in viscosity index and little if any change in viscosity. This mild operation is carried out at a pressure between about 200 and 2,000 p.s.i.g., at a temperature between about 450° and 750° F., at a space velocity between about 0.1 and 8.0. Any hydrogenation catalyst may be used such as nickel, cobalt, platinum and oxides and sulfides of group VI and group VII metals such as molybdenum, tungsten, nickel, cobalt, etc., oxides and sulfides or mixtures thereof. Porous supports may be used. Such procedure may be used to prepare an improved lubricating oil in accordance with our invention.

Another known method of hydrogenating lubricating oils is more severe than the above discussed hydrogen treatment. In this process the objective is not only to hydrogenate easily saturated materials such as olefins, but also to effect a more or less extensive hydrogenation of aromatics. In this type of process a moderate improvement in viscosity index and slight reduction in viscosity is also obtained, indicating a certain amount of hydro-cracking. This process is carried out in the presence of mixtures of a sulfide of a metal of the iron group mixed with a sulfide of a metal of group VI of the periodic system. These catalysts may be supported or unsupported on porous carriers. In the event a supported catalyst is employed, the carrier may be activated alumina, pumice, silica-alumina mixtures, etc. Pressures usually employed are about 1000 to 5000 p.s.i.g., temperatures between about 650° and 825° F. at a space velocity between about 0.1 and 4.0. This type of process may also be used in accordance with our invention.

A third type of lube oil hydrogen treatment is known in which extensive change takes place in the viscosity index and viscosity of the charge stock. In this type of process the same catalysts may be employed that are mentioned in connection with the second type of hydrogen treatment. Pressures employed are between about 1750 and 10,000 p.s.i.g.; temperatures are between about 735° and 825° F.; and space velocities are usually between 0.4 and 1.5. One aspect of this last mentioned type of process is the preparation of multigrade lubricating oils. In the event such a product is desired, the charge stock should have a viscosity index between about 60 and 100. We prefer to utilize as charge stock to the ionizing radiation a lubricating oil which has been subjected to a hydrogen treatment of the second or third type discussed above.

Certain aspects of the above described hydrogen treatments are described in United States patent application Serial No. 622,312, filed November 15, 1956, Beuther and Peterson, now Patent 2,917,448, and in United States patent application Serial No. 676,039, filed August 2, 1957, Beuther, Henke and McKinley, now Patent 2,960,458.

The hydrogenated lube oil stock may be subjected to the influence of the ionizing radiation in any desired manner. For instance, the lubricating oil may be pumped through a tube or pipe which is transparent to the ionizing radiations and which is exposed thereto. Alternatively, the hydrogenated lube oil stock may be caused to flow by gravity, preferably in the form of thin film over a surface which is subjected to the influence of the ionizing radiation. Another satisfactory method is to place the lube oil in reservoirs or pans and convey these reservoirs through the ionizing radiations by means of an endless

belt or the like. The exposure to the ionizing radiation should be kept within the limits described above, i.e. between about 0.001 and 10 watt hours per gram of lube oil stock and preferably between about 0.003 and 3.0 watt hours per gram. We have found that the viscosity of the lube oil stock begins to increase rapidly at above 10 watt hours per gram and therefore we prefer to keep the ionizing radiation exposure below this value and preferably between about .003 and 3 watt hours per gram. The radiation may be carried out at any desired temperature or pressure. Thus any temperature from 0° K. up to just below the decomposition temperature which usually is about 700° F. may be used. The pressure does not affect the reaction and therefore may vary from the lowest obtainable reduced pressure up to the highest obtainable pressure. As a practical matter we prefer to employ about ambient temperature and pressure.

Ionizing radiations can be obtained, for example, using radio isotopes, nuclear reactors or high energy particle accelerators. Examples of radio isotopes which can be used are cobalt 60 for gamma rays and strontium 90 for beta rays. Operating nuclear reactors of intermediate or full power size can be used as a source for either gamma rays or neutrons or both. Particle accelerators such as the cyclotron, bevatron, synchrotron, Van de Graaff or X-ray machines can also be used.

In some instances where it is desirable to expose the oil to fast or high energy neutrons only, and in the substantial absence of beta and gamma radiation, the irradiation can be conducted outside of the reactor using a collimated beam of fast neutrons. Such a collimated beam of fast neutrons can be obtained, for example, as described in U.S. Patent No. 2,708,656 to Enrico Fermi and Leo Szilard, by inserting a hollow shaft or tube into the central portion of the reactor. Gamma rays can be screened from the fast neutron beam by means of a sheet of bismuth metal extending across the path of the beam.

A neutron-free radiation source can be obtained directly from a homogeneous reactor by separating the radioactive fission gases, xenon and krypton, from the reactor core by conventional or modified gas-liquid separating means. A continuous supply of the radioactive fission gases could be obtained from such a reactor. The fission gases have

a very high intensity of beta and gamma radiation but a very short half life. These gases possess about one percent of the total fission energy. The gases are chemically inert and therefore would not form undesired side reaction products.

5

#### Example

A hydrotreated residuum, prepared in the manner described below, having a viscosity of 100 S.U.S. at 210° F. and an unhydrogenated residuum having substantially the same viscosity were compared before and after irradiation. The irradiation was carried out by pumping the sample of oil through a glass tube exposed to a beam of electrons from a 3-million volt Van de Graaff machine at a rate of 4 to 5 gallons per minute until the indicated irradiation exposure had been delivered. The properties of the hydrotreated residuum are given in column 1 of the following table. The properties of the non-hydrogenated residuum are given in column 5 of the accompanying table. The properties of the irradiated hydrotreated residuum are given in columns 2, 3 and 4 of the accompanying table while the properties of the irradiated non-hydrogenated residuum are given in column 6 of the accompanying table.

10 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000

A hydrotreated residuum, prepared in the manner described below, having a viscosity of 100 S.U.S. at 210° F. and an unhydrogenated residuum having substantially the same viscosity were compared before and after irradiation. The irradiation was carried out by pumping the sample of oil through a glass tube exposed to a beam of electrons from a 3-million volt Van de Graaff machine at a rate of 4 to 5 gallons per minute until the indicated irradiation exposure had been delivered. The properties of the hydrotreated residuum are given in column 1 of the following table. The properties of the non-hydrogenated residuum are given in column 5 of the accompanying table. The properties of the irradiated hydrotreated residuum are given in columns 2, 3 and 4 of the accompanying table while the properties of the irradiated non-hydrogenated residuum are given in column 6 of the accompanying table.

These various oil samples were then subjected to a modified Panel Coking Test as described in paragraph 4.5.9 of Specification MIL-L-9236A. The apparatus used for the Panel Coking Test is described in "Detailed Handbook on Test Procedures in Support of Turbojet and Turboprop Lubricants," March 1957, Wright Air Development Center. The modified procedure used in this example differs from that described in the reference only in that (1) only enough oil (which is often available only in small quantity) is placed in the reservoir to keep the sump at the required level during the test period, and (2) the edges of the panels are not scraped to remove coke.

The panel deposit weights listed in the table show clearly the advantages of the instant invention. The data in the table also show that the irradiation of the unhydrogenated oil resulted in a severe increase in deposit weight. Several of the control and test samples were also subjected to the MIL-L-9236A oxidation test as set forth in the table. The results of these oxidation tests show that the irradiated and hydrotreated oil was not

| Column Number                                                               | Hydrotreated Residuum<br>101 vis./210° F. |       |       |        | Unhydrogenated Residuum |       |
|-----------------------------------------------------------------------------|-------------------------------------------|-------|-------|--------|-------------------------|-------|
|                                                                             | 1                                         | 2     | 3     | 4      | 5                       | 6     |
| Irradiation Dosage (watt hours per gram)                                    | 0                                         | .0278 | 0.278 | 2.78   | 0                       | 0.278 |
| Inspections:                                                                |                                           |       |       |        |                         |       |
| Gravity, °API                                                               |                                           | 29.8  | 29.1  | 25.0   | 27.2                    | 27.1  |
| Viscosity, kinematic, cs.—                                                  |                                           |       |       |        |                         |       |
| 100° F.                                                                     | 243                                       | 246.8 | 324.8 | 14,904 | 244.5                   | 311.9 |
| 210° F.                                                                     | 20.81                                     | 21.03 | 25.79 | 583.5  | 19.91                   | 23.80 |
| Viscosity Index                                                             | 107                                       | 106   | 108   | 121    | 101                     | 103   |
| Color, D1500                                                                | 1.5                                       | 2     | 3.5   | 5.5    | 3                       | 3     |
| Flash, °F                                                                   | >550                                      | >550  | 515   | 420    | 565                     | 550   |
| Fire, °F                                                                    |                                           |       | 600   |        | 620                     | >600  |
| Pour, °F                                                                    | +5                                        | +5    | 0     | +20    | 0                       |       |
| Neutralization Value—                                                       |                                           |       |       |        |                         |       |
| Total Acid No. D664                                                         | 0.04                                      | 0.12  | 0.06  | 0.46   | 0.01                    | 0.08  |
| Panel Coking Test (700° F., 8 hrs.):                                        |                                           |       |       |        |                         |       |
| Coke deposit, mg.                                                           | a 1,238                                   | 84    | b 374 | 95     | c 90                    | d 362 |
| 500° F. Oxidation Test of Spec. MIL-L-9236A, 48 hrs., 500° F., 5 liters/hr. |                                           |       |       |        |                         |       |
| dry air per 100 ml. oil:                                                    |                                           |       |       |        |                         |       |
| Increase in 100° F., cs. vis., per cent                                     | 110                                       |       | 129   |        | 179                     | 236   |
| Increase in Total Acid No.                                                  | 3.48                                      |       | 3.11  |        | 3.87                    | 3.70  |
| Weight change of metals, mg./cm. <sup>2</sup>                               |                                           |       |       |        |                         |       |
| Mg                                                                          | +0.03                                     |       | -0.06 |        | +0.04                   | +0.04 |
| Al                                                                          | 0                                         |       | +0.01 |        | -0.21                   | 0     |
| Cu                                                                          | -0.01                                     |       | 0     |        | -0.01                   | -0.02 |
| Steel                                                                       | +0.03                                     |       | +0.01 |        | +0.03                   | +0.03 |
| Ag                                                                          | +0.01                                     |       | +0.01 |        | +0.03                   | +0.01 |
| Ti                                                                          | +0.01                                     |       | -0.01 |        | +0.03                   | -0.01 |

<sup>a</sup> Average of 5 tests. <sup>b</sup> Average of 4 tests. <sup>c</sup> Average of 13 tests. <sup>d</sup> Average of 2 tests.

(All tests were included in determining the average.)

harmfully affected in regard to its oxidation characteristics.

The hydrotreated oil used in the above example was obtained by subjecting a deasphaltered Ordovician residuum to treatment with hydrogen at a pressure of 3,000 p.s.i.g. at a temperature of 715° F., using a space velocity of 0.5, and an hydrogen recycle rate of 5,000 s.c.f./bbl. in the presence of a nickel-tungsten sulfide catalyst. The non-hydrogenated residuum used in the above example was obtained by subjecting a deasphaltered Ordovician residuum to treatment with aluminum chloride. The irradiations were carried out at approximately ambient temperature.

What we claim is:

1. The process for preparing a lubricating oil having a 15 relatively low tendency to deposit coke as determined by the Panel Coking Test, which process comprises subjecting a hydrogenated lubricating oil which has a viscosity between about 50 and 150 S.U.S. at 210° F. to ionizing

radiation of between about 0.001 and 10.0 watt hours per gram of hydrogenated lubricating oil.

2. The process for preparing a lubricating oil having a relatively low tendency to deposit coke as determined by the Panel Coking Test, which process comprises subjecting a hydrogenated lubricating oil which has a viscosity between about 50 and 150 S.U.S. at 210° F. to ionizing radiation of between about 0.001 and 10.0 watt hours per gram of hydrogenated lubricating oil at about 10 ambient temperature and pressure.

References Cited in the file of this patent

UNITED STATES PATENTS

|           |                        |                |
|-----------|------------------------|----------------|
| 2,905,606 | Long et al. -----      | Sept. 22, 1959 |
| 2,951,022 | Hartzband et al. ----- | Aug. 30, 1960  |
| 2,954,334 | Stoops et al. -----    | Sept. 27, 1960 |
| 2,990,350 | Natkin et al. -----    | June 27, 1961  |
| 3,043,759 | Read et al. -----      | July 10, 1962  |
| 3,058,896 | Nahin -----            | Oct. 16, 1962  |